

# United States Patent [19]

Burns

[11] 4,295,862

[45] Oct. 20, 1981

[54] MOTOR FUEL

[75] Inventor: Lyle D. Burns, Bartlesville, Okla.

[73] Assignee: Phillips Petroleum Company,  
Bartlesville, Okla.

[21] Appl. No.: 200,292

[22] Filed: Oct. 24, 1980

[51] Int. Cl.<sup>3</sup> ..... C10L 1/22

[52] U.S. Cl. ..... 44/72; 44/74;  
252/386

[58] Field of Search ..... 44/72, 74; 252/386

[56] References Cited

## U.S. PATENT DOCUMENTS

|           |         |                        |         |
|-----------|---------|------------------------|---------|
| 1,592,952 | 7/1926  | Martin                 |         |
| 1,940,096 | 12/1933 | Mueller-Cunradi et al. | 23/250  |
| 2,203,374 | 4/1940  | van Melsen             | 44/9    |
| 2,270,779 | 1/1942  | Berl                   | 260/603 |
| 2,333,294 | 11/1943 | Chenicek               | 44/72   |
| 2,881,061 | 4/1959  | Brennan et al.         | 44/63   |

|           |         |                 |       |
|-----------|---------|-----------------|-------|
| 2,910,352 | 10/1959 | Sweeney         | 44/68 |
| 3,009,793 | 11/1961 | Eckert et al.   | 44/69 |
| 3,133,952 | 5/1964  | Kline           | 44/74 |
| 3,706,541 | 12/1972 | Stournas et al. | 44/63 |

## OTHER PUBLICATIONS

T. A. Boyd, "Relative Effects of Some Nitrogen Compounds Upon Detonation in Engines", Sep. 1924, I & EC, 16 pp. 893-895.

Brown et al., "Mechanism of Aromatic Amine Antiknock Action", Oct., 1955, I & EC, 47 pp. 2141-2146.

Primary Examiner—Winston A. Douglas  
Assistant Examiner—Y. Harris-Smith

## ABSTRACT

Liquid hydrocarbon fuel compositions are provided containing antiknock quantities of ashless antiknock agents comprising selected acetylenic amine compounds.

6 Claims, No Drawings

## MOTOR FUEL

This invention relates to liquid hydrocarbon fuel compositions having improved antiknock properties. In one of its aspects, this invention relates more particularly to liquid hydrocarbon fuel compositions intended for use in internal combustion engines containing novel and effective ashless antiknock agents. In accordance with a further aspect, this invention relates to liquid hydrocarbon compositions containing antiknock quantities of ashless antiknock agents comprising selected acetylenic amine compounds.

Various antiknock agents have, heretofore, been suggested and employed for use in liquid hydrocarbon fuels, particularly in fuels employed in internal combustion engines. In such engines, it is highly desirable, from a stand point of economics that combustion of the fuel occurs at relatively high compression ratios. Such high compression ratios concomitantly necessitate the use of fuels having relatively high octane numbers to insure knock-free operation. Many antiknock agents have been proposed and/or used to improve the antiknock properties of hydrocarbon fuels used for internal combustion engines. In general, however, none of these antiknock additives have proved to be satisfactory in effectively raising the octane number of the fuel without also exhibiting other undesirable properties of varying importance. The phase-down of lead in gasoline as required by federal law and the banning of certain additives from use in unleaded gasoline has given impetus to continuation of a systematic study of the antiknock activity of ashless (non-metallic) compounds. The present invention is directed to the use of ashless (non-metallic) additives as antiknock agents for internal combustion fuels.

Accordingly, an object of this invention is to provide ashless hydrocarbon fuel compositions.

Another object of this invention is to provide ashless (non-metallic) antiknock additives for internal combustion engine fuels.

Another object of this invention is to provide hydrocarbon fuel compositions exhibiting improved antiknock properties.

Other objects, aspects as well as the several advantages of the invention will be apparent to those skilled in the art upon reading the specification and the appended claims.

In accordance with the present invention, new and improved liquid hydrocarbon fuel compositions are provided containing an antiknock quantity of ashless (non-metallic) additives comprising selected acetylenic amines.

The antiknock additives of the invention are known and can be prepared by processes known in the art.

Specific examples of ashless antiknock agents of the invention that can be used in internal combustion engine fuels include N-methylpropargylamine, N-benzyl-propargylamine, N-phenylpropargylamine, dipropargylamine, and N,N'-diethyl-2-butyne-1,4-diamine, and mixtures thereof. These compounds have suitable solubility and volatility characteristics to permit their application as additives for hydrocarbon fuels.

The antiknock additives of the invention are highly suited for use in fuels in view of their ashless characteristics. Naturally, the various compounds of the herein disclosed group do not possess exactly identical effectiveness, and the most advantageous concentration for each such compound will depend to some extent upon

the particular compound used. Also, the minimum effective inhibitor concentration can vary somewhat according to the specific nature of the hydrocarbon composition to which it is added.

The amounts of the antiknock agents of the invention added to the hydrocarbon fuels will be sufficient to improve the antiknock properties of the fuel. In general, these novel antiknock additives are employed in amounts from about 0.5 to about 10 percent (5000 to 100,000 parts per million), preferably from about 1 to about 5 percent (10,000 to 50,000 parts per million), by weight of the total weight of the fuel composition.

The motor fuels or gasolines into which the invention additives are incorporated are conventional motor fuel distillates boiling in the range of 70-420° F. (21.1°-216° C.). Gasolines or automotive fuels to which the described additives perform the functions described herein include substantially all grades of gasoline presently being employed in automotive and internal combustion aircraft engines. Generally automotive and aircraft gasolines contain both straight run and cracked stock with or without alkylated hydrocarbons, reformed hydrocarbons, and the like. Such gasolines can be prepared from saturated hydrocarbons, e.g., straight run stocks, alkylation products, and the like, with or without gum inhibitors, detergents, corrosion inhibitors, solvents, emulsifiers, and the like. The motor fuels are unleaded but can contain other conventional fuel additives such as antioxidants and the like.

## SPECIFIC EXAMPLE

The acetylenic amine derivatives N-methylpropargylamine (I), N-benzylpropargylamine (II), N-phenylpropargylamine (III), dipropargylamine (IV), and N,N'-diethyl-2-butyne-1,4-diamine (V) were dissolved singly at a concentration of 0.1 molar in clear (unleaded) FT-175 gasoline. The following table presents the characteristics of the FT-175.

## CHARACTERISTICS OF TEST GASOLINE

Description: Unleaded Kansas City Premium Pipeline Base Gasoline

| Designation              | FT-175   |
|--------------------------|----------|
| Reid Vapor Pressure, psi | 7.2      |
| API Gravity @ 60F        | 64.4     |
| <u>ASTM Distillation</u> |          |
| Vol % Evaporated         | Temp., F |
| IBP                      | 86       |
| 5                        | 115      |
| 10                       | 132      |
| 15                       | 145      |
| 20                       | 157      |
| 30                       | 178      |
| 40                       | 197      |
| 50                       | 213      |
| 60                       | 229      |
| 70                       | 250      |
| 80                       | 286      |
| 90                       | 353      |
| 95                       | 391      |
| EP                       | 428      |
| Lead Content, g/gal      | 0.005    |
| Sulfur Content, wt %     | 0.04     |
| Research Octane Number   | 91.5     |
| Motor Octane Number      | 83.9     |
| <u>Component</u>         | vol %    |
| Paraffins                | 69.03    |
| Olefins                  | 15.01    |
| Naphthenes               | 6.63     |
| Aromatics                |          |

-continued

|                               |       |
|-------------------------------|-------|
| Average Molecular Weight      | 101.3 |
| Atomic Ratio: Hydrogen/Carbon | 2.10  |
| Stoichiometric Air-Fuel Ratio | 14.89 |

Each gasoline was engine tested to determine its Research Octane Number (RON) according to ASTM D 2599-47. The following table presents the increase in RON over the untreated fuel produced by the addition of the selected acetylenic amine compounds.

| Compounds | Conc., wt. % | RON increase |
|-----------|--------------|--------------|
| I         | 1.0          | 0.7          |
| II        | 2.0          | 0.6          |
| III       | 1.8          | 1.2          |
| IV        | 1.3          | 0.3          |
| V         | 1.9          | 0.5          |

The efficacy of the novel ashless antiknock compounds of the present invention for improving the anti-knock properties of liquid hydrocarbon fuels will be apparent from the foregoing example and comparative data. It will be understood that the novel ashless anti-knock compounds of the present invention can be advantageously employed in any liquid hydrocarbon fuel composition which is suitable for use in a combustion engine regardless of the purpose for which the engine is designed.

20  
25  
304  
I claim:

1. An internal combustion fuel composition comprising a major proportion of a motor fuel containing a small but effective amount, sufficient to impart reduced knocking tendencies to said motor fuel, of an ashless antiknock additive selected from the group consisting of (I) N-methylpropargylamine, (II) N-benzylpropargylamine, (III) N-phenylpropargylamine, (IV) dipropargylamine, and (V) N,N'-diethyl-2-butyne-1,4-diamine.

2. A composition according to claim 1 wherein the motor fuel contains from about 0.5 to about 10 weight percent of said additives.

3. A composition according to claim 1 wherein the motor fuel is a distillate boiling in the range of about 70° F. to about 420° F. (21.1°-216° C.).

4. A gasoline composition containing an antiknock quantity of at least one ashless antiknock additive of the group consisting of N-methylpropargylamine (I), N-benzylpropargylamine (II), N-phenylpropargylamine (III), dipropargylamine (IV), and N,N'-diethyl-2-butyne-1,4-diamine.

5. The composition of claim 4 containing from about 0.5 to about 10 percent by weight of the antiknock additive.

6. The composition of claim 4 containing from about 1 to about 5 percent by weight of the antiknock additive.

\* \* \* \* \*

35

40

45

50

55

60

65